

## UNITED STATES PATENT OFFICE

2,204,230

## AZO DYES

Swanie S. Rossander and Chiles E. Sparks, Wilmington, Del., assignors to E. I. du Pont de Nemours & Company, Wilmington, Del., a corporation of Delaware

No Drawing. Application March 29, 1939,  
Serial No. 264,837

18 Claims. (Cl. 260—144)

This invention relates to azo dyes, to direct dyes, to dyes after-treated with formaldehyde, and to metalized dyes.

Direct azo dyes are those which dye the cloth directly from a water bath without subsequent treatment to bring out the color. Many examples of such direct dyes are recorded in the literature of the trade. These direct colors are generally substantive to cotton and other forms 10 of cellulose and regenerated cellulose, giving bright shades, but having only moderate fastness to light. These direct colors show considerable loss in strength and impart an undesirable stain to associated uncolored or differently colored 15 fibers when they are washed. Direct colors with good washing fastness, and which will not stain associated fibers are desired by the trade because of their low cost and ease of application. In order to provide dyes which do not have poor 20 fastness to washing the art has been forced to use the developed colors, wherein an intermediate, usually a direct dye, is azotized on the fiber and developed with suitable coupling compounds. These, so-called developed or diazo colors are 25 generally faster to washing than the corresponding direct colors, but they are duller, more costly, more costly to apply as such dyeing operations require much labor and the dyeings change shade during development.

It is an object of this invention to provide a class of colors having the simplicity of application and constant, bright shade of the direct colors, and washing fastness superior to the direct colors. Another object of the invention is 35 to provide methods of applying the colors, and of increasing their light fastness.

The objects of the invention are accomplished in general by applying to the material to be dyed, the direct polyazo dyes represented by the formula

40



and after-treating the dyed fabric with formaldehyde, formaldehyde and a soluble metal salt, or 45 a soluble metal salt.

The symbol A in the foregoing formula is a metadihydroxy benzene represented by the formula



in which R is one of a group consisting of hydrogen, alkyl, alkoxy, aralkyl, hydroxy, amino, halogen, nitrile, carboxy and sulfonic acid. 10

The symbols X are diamino-diphenylene compounds in which the amino groups are in meta or para positions to the bridged carbons and are 15 represented by the formula



in which B is one of a group consisting of —O—, 20 —S—, —NH—, —NHCONH—, —NHCSNH—, —CONH—, —CONH(CH2)mNHCO—, —HC=CH—, 25



wherein the —NHCO— groups are meta or para to each other, —O(CH2)mO—, —S(CH2)mS—, 30 —N=N—, 35



and —(CH2)m—, n is an integer 1 or 2, m is 2 to 7, R1 is at least one of a group consisting of hydrogen, alkyl, alkoxy and halogen and where there is more than one R1 the substituents may be alike or different. R2 is one or more than one of said group hydrogen, alkyl, alkoxy and halogen in any combination thereof. In cases where n is 1 in the group —(B)n— the symbol X stands for a diamino diphenyl, such as benzidine, or one of the indicated derivatives thereof. 40 45

The symbol Y is an amino naphthol sulfonic acid represented by the formula



in which amino is in the 1 or 2 position, R<sub>3</sub> is one of a group consisting of hydrogen, alkyl, 10 alkoxy, aralkyl, nitro, halogen, nitrile, sulfonic acid and carboxy.

The symbol Z is a compound of the benzene series represented by the formula



20 in which R<sub>5</sub> is one of a group consisting of hydrogen, alkyl, alkoxy, phenyl-alkyl, hydroxy, amino, alkylated amino, halogen, CN and sulfonic acid, and each R<sub>6</sub> is one of a group consisting of amino, hydroxy and alkylated amino. The R<sub>4</sub> groups may be alike or unlike.

In general R, R<sub>1</sub>, R<sub>2</sub>, R<sub>3</sub> and R<sub>5</sub> may be substituted in any open position of the aryl nuclei, except where the formulas indicate that the positions of such substituents are fixed. The term 30 alkylated amino as used in the specification and claims refers to the secondary or tertiary group



in which X<sub>1</sub> and X<sub>2</sub> may be alike or different groups, X<sub>1</sub> is alkyl, phenyl-alkyl or hydroxy alkyl and X<sub>2</sub> is hydrogen, alkyl, phenyl-alkyl or hydroxy alkyl. As illustrations of alkylated amino groups are mentioned the groups —N(CH<sub>3</sub>)<sub>2</sub>, —NH-CH<sub>3</sub>, —NCH<sub>3</sub>(C<sub>2</sub>H<sub>5</sub>OH), —NCH<sub>3</sub>(C<sub>2</sub>H<sub>5</sub>), —NH(C<sub>2</sub>H<sub>5</sub>OH), —N(C<sub>2</sub>H<sub>5</sub>OH)—C(H<sub>2</sub>C<sub>6</sub>H<sub>5</sub>), —NH-C<sub>6</sub>H<sub>5</sub> and —N(C<sub>6</sub>H<sub>5</sub>)<sub>2</sub>. Alkyl in the specification and claims refers to straight and branched chain aliphatic groups having 1 to 4 carbons, alkoxy refers to the corresponding alkoxy groups and halogen refers to any of the halogens.

The compounds of the invention may be made 50 in general by coupling one mol equivalent of the diamino compound Z to one mol equivalent of the diazo of the naphthol amino sulfonic acid compound Y, isolating the resulting compound Y-Z and then dissolving it in basic solution. Two mol 55 equivalents of the diamino diphenyl compound X are then tetrazotized and coupled in basic medium with the one mol equivalent of the compound Y-Z. This produces a basic tetrazo solution of the compound X-Y-Z-X. This compound 60 is then coupled in basic medium with two mol equivalents of the dihydroxy phenyl compound A and the product A-X-Y-Z-X-A is isolated by appropriate means, as by salting out and filtering.

65 Dyeings may be made in general by dissolving the products A-X-Y-Z-X-A in a suitable solvent such as water. Dyeing assistants and other compounds which are necessary or desirable to produce dyeings on fabrics can be added to the 70 solution to make the dyebath. The material to be dyed is then immersed in the dyebath which may have been previously heated. When dyed the material is after-treated in a bath containing formaldehyde until a formaldehyde 75 pound or complex is formed. The resulting dye-

ings have excellent washing fastness. If improved light fastness is desired, this can be obtained by additionally treating the dyeing in a bath containing a soluble metal salt, such as copper sulfate.

The invention will be more fully set forth in the following more detailed description which includes examples that are given as illustrative embodiments of the invention and not as limitations thereof.

5

10

#### EXAMPLE 1

Slurry 34.1 parts of the mono-sodium salt of 2-amino-8-naphthol-3,6-disulfonic acid with 300 parts of water. Add approximately 4.0 parts of sodium hydroxide to the slurry and stir until a complete solution is obtained which is faintly alkaline to Brilliant Yellow paper. Cool to 0° C. with ice and add 14.5 parts of 100% hydrochloric acid as a 30% solution. Slowly add to this solution 6.9 parts of 100% sodium nitrite as a 30% solution. Maintain a slight excess of nitrite in the mixture for 15 minutes whilst it is cooled to 0-5° C. Finally balance to a very faint or negative nitrite test by the addition of a neutral solution of the diazo component.

20

Dissolve 10.8 parts of 1,3-diamino-benzene in 200 parts of water at 50-60° C. Cool to 25° C. with ice and add the cooled mixture rapidly to the above described diazo of 2-amino-8-naphthol-3,6-disulfonic acid. Stir 5 minutes then add slowly during 30 minutes 11.0 parts of sodium carbonate and finally stir the mixture for two hours. The suspension is produced which is neutral to Congo red papers and is neutral to slightly alkaline to Brilliant Yellow paper. There should be an excess of 1,3-diamino-benzene present and the mixture should give no test for diazo.

30

Make the above described suspension acid to Congo red papers by adding 73.0 parts of 100% hydrochloric acid as a 30% solution. Salt slowly (25%) with sodium chloride. Stir one hour and filter.

35

Dissolve the filter cake in 1000 parts of water at 40°-50° C. by the addition of approximately 32.0 parts of sodium carbonate and then cool to 20° C. by adding ice.

40

Slurry 36.8 parts of 4,4'-diamino-diphenyl with 1000 parts of water. Add 37.0 parts of 100% hydrochloric acid as a 30% solution and cool to 0° C. with ice. Tetrazotize at 0-5° C. for 30-40 minutes by adding 27.6 parts of 100% sodium nitrite as a 30% solution. The tetrazo should be free of insoluble matter and there should be an excess nitrite.

45

Make the above described tetrazo distinctly alkaline to Brilliant Yellow by adding 64 parts of 100% sodium carbonate as a 5% solution. While maintaining a temperature of 0-5° add the alkaline solution of 2-amino-8-naphthol-3,6-disulfonic acid to 1,3-diamino-benzene slowly to the cold alkaline tetrazo until there is no test for 4,4'-diamino-diphenyl tetrazo. It is desirable to remove a portion of the tetrazo, say 5 to 10% before the latter addition is made so that the portion can be used to balance the coupling.

55

Immediately upon the disappearance of the 4,4'-diamino-diphenyl tetrazo, add rapidly 33 parts of 1,3-dihydroxy-benzene and stir the mixture for one hour. Keep the suspension alkaline to Brilliant Yellow and maintain an excess of 1,3-dihydroxy-benzene.

60

After stirring, the suspension was heated to 70°-80° C., salted slowly (10%) with sodium chloride, filtered and dried in an oven at 80-85° C. The dry powder was deep brown in appearance.

70

75

The compound is represented by the formula



A fabric of regenerated cellulose rayon was dyed with the dye and after-treated as follows.

15 A solution of the dye was made by dissolving 0.2 gram of the dye in 50 cc. of water at 190°-200° F. and adding .04 gram of sodium carbonate to assist the solution. The bath was diluted with hot water at 160° F. to a total volume of 500 cc. whilst stirring and 40 cc. of a 10% solution of Glauber's salt were added. A 10 gram piece of regenerated cellulose rayon was wet out with water, squeezed partially dry and entered into the dyebath. The temperature of the dyebath was raised to 180°-190° F. during a period of fifteen minutes and was held at that temperature for one hour. The dyeings were stirred at frequent intervals. At the end of one hour the dyeing was removed and rinsed in cold water.

#### *After-treatment in a fresh bath*

35 The rinsed dyeing from the above operation was entered into 500 cc. of water at 130°-140° F. and approximately 10 cc. of 10% formaldehyde (25 cc. of approximately 37% formaldehyde by weight diluted to 250 cc. with water) were added. The bath was held at this temperature for twenty minutes. The dyeing was then removed, rinsed and dried.

#### *After-treatment in the dye bath*

An alternative after-treating process which is the preferred procedure because of its economy and ease of application was carried out as follows:

50 A dyeing with a deep brown shade was obtained which showed excellent fastness to washing. The fastness to washing was better than the direct dyeing.

**EXAMPLE 2**

55 Slurry 42.5 parts of 4,4'-diamino-azobenzenes with 1000 parts of water. Add 37 parts of 100% hydrochloric acid as a 30% solution. Ice to 0° C. Tetrazotize at 0-5° C. for 30-40 minutes with 27.6 parts of 100% sodium nitrite as a 30% solution. The tetrazo should be free of insoluble matter and there should be present an excess of nitrite. Balance to a very faint excess of nitrite.

Add approximately 100 parts crystalline sodium acetate to the tetrazo. The tetrazo solution

should be neutral to Congo red paper. To the neutralized tetrazo, a slightly alkaline solution of the mono-azo product, 2-amino-8-naphthol-3,6-disulfonic acid-1,3-diamino-benzene, prepared as in Example 1, is added until there is no test for 4,4'-diamino-azo-benzene tetrazo.

Immediately upon the disappearance of the 4,4'-diamino-azo-benzene tetrazo, add rapidly 33 parts of 1,3-dihydroxy-benzene. Add slowly approximately 60 parts of sodium carbonate to make the suspension alkaline to Brilliant Yellow. There should be an excess of 1,3-dihydroxy-benzene.

Heat the suspension to 70°-80° C. Salt slowly 10% with sodium chloride. Filter. Dry at 80°-85° C. in an oven. The dry powder was a deep brown in appearance.

The dye is represented by the formula



Regenerated cellulose rayon was dyed with the dye and after-treated as described in Example 1. A dyeing with a deep brown shade was obtained which showed good fastness to washing. The dyeing had better fastness to washing than the direct dyeing.

### EXAMPLE 3

A product represented by the following formula was obtained by substituting 48.5 parts of di(3-aminophenyl) urea for 36.8 parts of 4,4'-diaminodiphenyl in Example 1. 60



Regenerated cellulose rayon was dyed with the dye and after-treated as in Example 1. A dyeing with a yellow brown shade was obtained which showed good fastness to washing. The washing fastness was better than the direct dyeing.

It is to be understood that modifications in the methods of preparing the compounds can be made and the invention is not limited by the details particularized in the examples. The compounds can be prepared by suitable modifications of the methods set forth without departing from the invention as will be understood by those skilled in the art.

The following are additional illustrations of the invention. These products were prepared by methods similar to those recited in the foregoing examples. The most applicable variations in the method of making these compounds is apparent to those skilled in the art for any given example, wherever a variation is desirable. The direct dyeings with the colors on regenerated cellulose rayon and after-treatment with formaldehyde gave bright shades which were comparable in brightness and washing fastness to those produced in the foregoing examples.

As other illustrations of meta-dihydroxy benzenes which may be used as the component A are mentioned:

3,5-dihydroxy toluene,  
3,5-dihydroxy anisole,  
3,5-dihydroxy benzoic acid,  
1,3-dihydroxy benzene-5-sulfonic acid,  
1,3-dihydroxy-5-amino benzene,  
1,3-dihydroxy-5-chloro-benzene,  
1,3-dihydroxy-5-bromo-benzene,  
1,3,5-trihydroxy benzene,  
1,3-dihydroxy-5-benzo-nitrile and  
1-benzyl-3,5-dihydroxy benzene.

As other illustrations of Y compounds the following naphthalene derivatives are mentioned:

2-amino-3-methyl-5-hydroxy-7-sulfonic acid,  
2-amino-3-methoxy-5-hydroxy-7-sulfonic acid,  
2-amino-3-benzyl-5-hydroxy-7-sulfonic acid,  
2-amino-3-nitro-5-hydroxy-7-sulfonic acid,  
2-amino-3-chloro-5-hydroxy-7-sulfonic acid,  
2-amino-3-bromo-5-hydroxy-7-sulfonic acid,  
2-amino-3-nitrile-5-hydroxy-7-sulfonic acid,  
2-amino-3-carboxy-5-hydroxy-7-sulfonic acid,  
1- and 2-amino-8-naphthol-6-sulfonic acids,

| Example | Constitution                                                                                                                                                                                                                                   | Shade            |
|---------|------------------------------------------------------------------------------------------------------------------------------------------------------------------------------------------------------------------------------------------------|------------------|
| 30 4    | 1,3-dihydroxybenzene ← 4,4'-diamino-diphenyl → 2-amino-8-naphthol-3,6-disulfonic acid → 1,3-dihydroxybenzene ← 4,4'-diamino-diphenyl → 1,3-dihydroxybenzene.                                                                                   | Brown. 30        |
| 5       | 3,5-dihydroxy-toluene ← 4,4'-diamino-diphenyl → 2-amino-8-naphthol-3,6-disulfonic acid → 1,3-diaminobenzene ← 4,4'-diamino-diphenyl → 3,5-dihydroxy-toluene.                                                                                   | Do.              |
| 6       | 1,3-dihydroxybenzene ← 4,4'-diamino-diphenyl → 1-amino-8-naphthol-3,6-disulfonic acid → 1,3-diaminobenzene ← 4,4'-diamino-diphenyl → dihydroxy-benzene.                                                                                        | Do.              |
| 7       | 1,3-dihydroxybenzene ← 4,4'-diamino-diphenyl → 2-amino-5-naphthol-7-sulfonic acid → 1,3-diaminobenzene ← 4,4'-diamino-diphenyl → 1,3-dihydroxy-benzene.                                                                                        | Do.              |
| 35 8    | 1,3-dihydroxybenzene ← 4,4'-diamino-diphenyl → 1-amino-5-naphthol-7-sulfonic acid → 1,3-diaminobenzene ← 4,4'-diamino-diphenyl → 1,3-dihydroxy-benzene.                                                                                        | Do. 35           |
| 9       | 1,3-dihydroxybenzene ← 4,4'-diamino-diphenyl → 2-amino-8-naphthol-6-sulfonic acid → 1,3-diaminobenzene ← 4,4'-diamino-diphenyl → 1,3-dihydroxy-benzene.                                                                                        | Do.              |
| 10      | 1,3-dihydroxybenzene ← 4,4'-diamino-stilbene → 2-amino-8-naphthol-3,6-disulfonic acid → 1,3-diaminobenzene ← 4,4'-diamino-stilbene → 1,3-dihydroxy-benzene.                                                                                    | Do.              |
| 11      | 1,3-dihydroxybenzene ← 3,3'-diamino-azoxy-benzene → 2-amino-8-naphthol-3,6-disulfonic acid → 1,3-diaminobenzene ← 3,3'-diamino-azoxy-benzene → 1,3-dihydroxybenzene.                                                                           | Yellow brown. 40 |
| 40 12   | 1,3-dihydroxybenzene ← 4,4'-diamino-diphenyl → 2-amino-8-naphthol-3,6-disulfonic acid → 5-methoxy-1,3-dihydroxy-benzene.                                                                                                                       | Brown. Do.       |
| 13      | 1,3-dihydroxybenzene ← 4,4'-diamino-diphenyl → 2-amino-8-naphthol-3,6-disulfonic acid → 1,3-diamino-4-methyl-benzene ← 4,4'-diamino-diphenyl → 1,3-dihydroxybenzene.                                                                           | Do.              |
| 14      | 1,3-dihydroxybenzene ← 3,3'-diamino-azoxy-benzene → 2-amino-8-naphthol-3,6-disulfonic acid → 1,3-dihydroxybenzene ← 3,3'-diamino-azoxy-benzene → 1,3-dihydroxybenzene.                                                                         | Do.              |
| 15      | 1,3-dihydroxybenzene ← (4,4'-diamino-diphenyl-amino-2'-sulfonic acid) → 2-amino-8-naphthol-3,6-disulfonic acid → 1,3-diaminobenzene ← (4,4'-diamino-diphenyl-amino-2'-sulfonic acid) → 1,3-dihydroxybenzene.                                   | Do. 45           |
| 16      | 1,3-dihydroxybenzene ← 2,2'-dichloro-4,4'-diamino-diphenyl → 2-amino-8-naphthol-3,6-disulfonic acid → 1,3-diaminobenzene ← 2,2'-dichloro-4,4'-diamino-diphenyl → 1,3-dihydroxybenzene.                                                         | Do.              |
| 17      | 1,3-dihydroxybenzene ← (3-(4'-aminobenzoyl-amino)-1-aminobenzene) → 2-amino-8-naphthol-3,6-disulfonic acid → 1,3-diaminobenzene ← (3-(4'-aminobenzoyl-amino)-1-aminobenzene) → 1,3-dihydroxybenzene.                                           | Do.              |
| 18      | 1,3-dihydroxybenzene ← (1,3-di(4'-amino-benzoyl-amino) benzene) → 2-amino-8-naphthol-3,6-disulfonic acid → 1,3-diaminobenzene ← (1,3-di(4'-amino-benzoyl-amino) benzene) → 1,3-dihydroxybenzene.                                               | Yellow brown. 50 |
| 50 19   | 1,3-dihydroxybenzene ← 1,2-di(4'-amino-benzoyl-amino) ethane → 2-amino-8-naphthol-3,6-disulfonic acid → 1,3-diaminobenzene ← (4-(4'-amino-2-methyl-phenyl) urea) → 1,3-dihydroxybenzene.                                                       | Brown. Do.       |
| 20      | 1,3-dihydroxybenzene ← (4-(4'-amino-2-methyl-phenyl) urea) → 2-amino-8-naphthol-3,6-disulfonic acid → 1,3-diaminobenzene ← (4-(4'-amino-2-methyl-phenyl) urea) → 1,3-dihydroxybenzene.                                                         | Do.              |
| 21      | 1,3-dihydroxybenzene ← (4-(4'-amino-5-methyl-1-amino-benzene)) → 2-amino-8-naphthol-3,6-disulfonic acid → 1,3-diaminobenzene ← (4-(4'-amino-5-methyl-1-amino-benzene)) → 1,3-dihydroxybenzene.                                                 | Do.              |
| 55 22   | 1,3-dihydroxybenzene ← 4,4'-diamino-2,2'-dimethyl-diphenyl-methane → 2-amino-8-naphthol-3,6-disulfonic acid → 1,3-diaminobenzene ← 4,4'-diamino-2,2'-dimethyl-diphenyl-methane → 1,3-dihydroxybenzene.                                         | Yellow brown. 55 |
| 23      | 1,3-dihydroxybenzene ← 4,4'-diamino-diphenyl-sulfide → 2-amino-8-naphthol-3,6-disulfonic acid → 1,3-diaminobenzene ← 4,4'-diamino-diphenyl-sulfide → 1,3-dihydroxybenzene.                                                                     | Brown.           |
| 24      | 1,3-dihydroxybenzene ← 4,4'-diamino-diphenylamine → 2-amino-8-naphthol-3,6-disulfonic acid → 1,3-diaminobenzene ← 4,4'-diamino-diphenylamine → 1,3-dihydroxybenzene.                                                                           | Do.              |
| 25      | 1,3-dihydroxybenzene ← ((4,4'-diamine benzene) → (2-methoxy-5-methyl-1-amino-benzene)) → 2-amino-8-naphthol-3,6-disulfonic acid → 1,3-diaminobenzene ← ((4,4'-diamine benzene) → (2-methoxy-5-methyl-1-amino-benzene)) → 1,3-dihydroxybenzene. | Do.              |
| 60 26   | 1,3-dihydroxybenzene ← 4,4'-diamino-diphenyl → 2-amino-8-naphthol-3,6-disulfonic-acid → 1,3-diaminobenzene-4-sulfonic-acid ← 4,4'-diamino-diphenyl → 1,3-dihydroxybenzene.                                                                     | Do. 60           |
| 27      | 1,3-dihydroxybenzene ← 4,4'-diamino-diphenyl → 2-amino-8-naphthol-3,6-disulfonic acid → 1,3-diamino-4-chloro-benzene ← 4,4'-diamino-diphenyl → 1,3-dihydroxybenzene.                                                                           | Do.              |
| 28      | 1,3-dihydroxybenzene ← 4,4'-diamino-diphenyl → 2-amino-8-naphthol-3,6-disulfonic-acid → 1,3-diaminobenzene ← di(4-amino-2-methyl-phenyl)urea → 1,3-dihydroxybenzene.                                                                           | Do.              |
| 29      | 1,3-dihydroxybenzene ← 1,2-di(4'-amino-phenoxo)ethane → 2-amino-8-naphthol-3,6-di-sulfonic-acid → 1,3-diaminobenzene ← 1,2-di(4'-amino-phenoxo)ethane → 1,3-dihydroxybenzene.                                                                  | Do.              |
| 65 30   | 1,3-dihydroxybenzene ← 4,4'-diamino-diphenyl-ether → 2-amino-8-naphthol-3,6-disulfonic-acid → 1,3-diaminobenzene ← 4,4'-diamino-diphenyl-ether → 1,3-dihydroxybenzene.                                                                         | Do. 65           |
| 31      | 1,3-dihydroxy-5-methyl-benzene ← 4,4'-diamino-diphenyl → 2-amino-8-naphthol-3,6-disulfonic-acid → 1,3-diaminobenzene ← 4,4'-diamino-diphenyl → 1,3-dihydroxy-5-methyl-benzene.                                                                 | Do.              |
| 32      | 1,3-dihydroxybenzene ← 4,4'-diamino-diphenyl → 2-amino-8-naphthol-3,6-disulfonic-acid → 1,3-diamino-4-benzene-sulfonic-acid ← 4,4'-diamino-diphenyl → 1,3-dihydroxybenzene.                                                                    | Do.              |
| 33      | 1,3-dihydroxybenzene ← 4,4'-diamino-diphenyl → 2-amino-8-naphthol-3,6-disulfonic-acid → 1,3-diamino-4-chloro-benzene ← 4,4'-diamino-diphenyl → 1,3-dihydroxybenzene.                                                                           | Do.              |
| 70 34   | 1,3-dihydroxybenzene ← 4,4'-diamino-diphenyl-oxide → 2-amino-8-naphthol-3,6-disulfonic-acid → 1,3-diaminobenzene ← 4,4'-diamino-diphenyl-oxide → 1,3-dihydroxybenzene.                                                                         | Do. 70           |
| 35      | 1,3-dihydroxybenzene ← 1,2-di(4'-amino-phenoxo)ethane → 2-amino-8-naphthol-3,6-disulfonic-acid → 1,3-diaminobenzene ← 1,2-di(4'-amino-phenoxo)ethane → 1,3-dihydroxybenzene.                                                                   | Do.              |

- 1- and 2-amino-7-naphthol-5-sulfonic acids,  
 1- and 2-amino-3-methyl-8-naphthol-6-sulfonic acids,  
 1- and 2-amino-3-nitro-8-naphthol-6-sulfonic acids, and  
 5 2-amino-3-carboxy-8-hydroxy-6-sulfonic acid.

As other illustrations of Z compounds are mentioned:

- 10 1,3-dihydroxy-5-benzo-nitrile,  
 1,3,5-trihydroxy benzene,  
 1,2,4-triamino benzene,  
 1-dimethylamino-2,4-diamino benzene,  
 1-methylamino-3,5-diamino-benzene,  
 15 3,5-di(ethyl amino) phenol,  
 1-(methyl amino)-3-amino benzene,  
 1,3-di(ethyl amino) benzene,  
 1-hydroxy-3-amino benzene,  
 1,3-di(ethyl amino) benzene,  
 20 1,3-dihydroxy-benzene-5-sulfonic acid,  
 1,3-dihydroxy-5-methyl-benzene and  
 2,4-diamino benzoic acid.

As other illustrations of X compounds are mentioned:

- 25 4,4'-diamino-3,3'-dimethyl-diphenyl,  
 2,2' - dichloro - 4,4' - diamino - 3,3' - dimethyl-diphenyl,  
 4,4'-diamino-3,3'-dimethyl-diphenyl-oxide,  
 30 4,4'-diamino-3,3'-dimethyl-diphenyl-sulfide,  
 4,4'-diamino-2,2'-dimethyl-diphenyl-amine,  
 di(2-methyl-5-amino-phenyl) urea,  
 di(4-amino-2-methoxy-phenyl) urea,  
 di(4-amino-phenyl) thio-urea,  
 35 4-(4'-amino-benzoyl-amino)-3-methyl-1-amino-benzene,  
 1,3-di(4-amino-benzoyl-amino) propane,  
 1,3-di(4'-amino-benzoyl-amino) - 4 - methyl-benzene,  
 40 1,2-di(4'-amino-2'-methoxy-phenoxy) ethane,  
 1,2-di(4'-amino-2'-methyl-phenoxy) ethane,  
 1,2-di(4'-amino-2'-chloro-phenoxy) ethane,  
 1,2-di(3'-amino-phenoxy) ethane,  
 1,3-di(4'-amino-phenoxy) propane,  
 45 1,3-di(4'-amino-phenoxy) heptane,  
 1,2-di(4'-amino-phenyl-thio) ethane,  
 1,3-di(4'-amino-phenyl-thio) propane,  
 4,4'-diamino-azoxy-benzene,  
 4,4'-diamino-diphenyl-ethane,  
 50 1,6-di(4'-amino-benzoyl-amino) hexane and  
 1,6-di(4'-amino-benzoyl-amino) heptane.

Deeper shades and improvement in the light fastness of the dyeings are produced by after-treatment of these colors with water soluble metal salts such as copper sulfate. For example the after-coppering operation may be carried out similarly to either of the procedures outlined in Example 1 for the after-treatment with formaldehyde, by using a solution containing a 5% solution of hydrated cupric sulfate equivalent in amount to the formaldehyde.

The after-treatment with metal salts may be allowed to continue for twenty minutes or for such other time as is necessary to metallize the dyeing, at the end of which time the treated dyeings are removed, rinsed and dried. The after-cooperating may replace the formaldehyde treatment, but it is preferable to after-treat with both formaldehyde and the metal salt where improvement in light-fastness is desired.

After-treatment with both formaldehyde and metal salts may be done either in the dye bath or in fresh baths. When a fresh formaldehyde bath is used and the dyeing is treated for a sufficient time to form the formaldehyde compound, the

metal salt may be added and the treatment continued for another interval of time. The dyeings are then removed, rinsed and dried. Similar results are obtained by reversing the order of adding the after-treating reagents, that is by adding the solution of metal salt first, treating for the necessary time and then adding the formaldehyde solution. After about twenty minutes the dyeings are removed, rinsed and dried.

The described method of dyeing is typical but it is to be understood that the invention is not limited to the precise concentrations, temperatures and times of treatment specified since these details can be variously modified as will be understood by those skilled in the art. For example, the after-treatments with formaldehyde or metal-salts may be carried on for longer or shorter periods and at higher or lower temperatures than those specified in the illustrations. Any treatment which will form a formaldehyde complex with the dyeing or a metal complex with the dyeing, as the case may be, produces the improved results. The exact composition of the described formaldehyde and metal complexes is unknown to us, but from our investigations it is our present belief that formaldehyde and metal complexes are formed.

Water-soluble salts of various metals can be used for metallizing the dyeings, those having atomic weights between 50 and 65 being the most suitable. As examples of such metals copper, chromium, nickel, cobalt and iron are mentioned. Either water-soluble salts of inorganic or organic acids can be used, such as sulfates, halides, formates and acetates, for example copper sulfate, nickel sulfate, chromium chloride, copper formate, copper acetate and many other water-soluble metal salts of inorganic and organic acids.

The invention provides bright dyeings having washing fastness equal to and in some cases superior to the diazo colors. The dyeings made in accordance with the invention are commonly produced more conveniently and more economically than the diazo colors since in a formaldehyde-treated direct dyeing only one bath is required, the dyeing operations are simple and no change of shade is encountered; whereas in a diazo dyeing at least two baths are required, a change of shade is produced and the dyeing is a complicated procedure. The dyes may be made in the form of the acid salts of any of the alkali metals by using an appropriate base of the desired alkali metal for neutralization.

Water-soluble salts of various metals can be used for metallizing the dyeings, those having atomic weights between 50 and 65 being the most suitable. As examples of such metals, copper, chromium, nickel, cobalt and iron are mentioned. Either water-soluble salts of inorganic or organic acids can be used, such as sulfates, halides, formates and acetates, for example, copper sulfate, nickel sulfate, chromium chloride, copper formate, copper acetate and many other water-soluble metal salts of inorganic and organic acids.

Since from the foregoing description of the invention it will be apparent to those skilled in the art that various other embodiments of the invention may be made without departing from the spirit and scope thereof, it is to be understood that the invention is not limited to the specific illustrations disclosed.

We claim:

1. A compound represented by the formula



in which A is the residue after coupling of a meta-dihydroxy benzene represented by the formula

5



in which R is one of a group consisting of hydrogen, alkyl, alkoxy, aralkyl, hydroxy, amino, halogen, nitrile, carboxy and sulfonic acid; each X is the residue after tetrazotization of a diphenylene diamine in which the amino groups are in meta or para positions to the bridged carbons and are represented by the formula

20



25

in which B is one of a group consisting of —O—, —S—, —NH—, —NHCONH—, —NHCSNH—, —CONH—, —(CONH(CH2)mNHCO)—, —HC=CH—

25



30

wherein the —NHCO— groups are meta or para to each other, —O(CH2)mO—, —S(CH2)mS—, —N=N—,

35



40

and —(CH2)m—, n is an integer not greater than 2, m is 2 to 7, R1 and R2 are each from the group consisting of hydrogen, alkyl, alkoxy and halogen; Y is the residue of an amino naphthol sulfonic acid represented by the formula

45



50

in which amino is in one of the positions 1 and 2 and R3 is one of a group consisting of hydrogen, alkyl, alkoxy, aralkyl, nitro, halogen, nitrile, sul-

55

fonic acid and carboxy; and Z is the residue of a compound represented by the formula

60



65

in which R5 is one of a group consisting of hydrogen, alkyl, alkoxy, phenyl-alkoxy, hydroxy, amino, alkylated amino, halogen, CN and sulfonic acid and the R4 groups are like or different members of a group consisting of amino, alkylated amino and hydroxy.

2. A compound represented by the formula

70



75

in which X is the residue after tetrazotization of a diphenylene diamine compound in which the amino groups are in meta or para positions to the

bridged carbons and are represented by the formula



5

in which B is one of a group consisting of —O—, —S—, —NH—, —NHCONH—, —NHCSNH—, —CONH—, —CONH(CH2)mNHCO—, —HC=CH—



15

wherein the —NHCO— groups are meta or para to each other, —O(CH2)mO—, —S(CH2)mS—, —N=N—,



20

and —(CH2)m—, n is an integer not greater than 2, m is 2 to 7, R1 is from the group consisting of hydrogen, alkyl, alkoxy and halogen and R2 is from the group consisting of hydrogen, alkyl, alkoxy and halogen; Y is the residue of an amino naphthol sulfonic acid represented by the formula



30

in which amino is in one of the positions 1 and 2 and R3 is one of a group consisting of hydrogen, alkyl, alkoxy, aralkyl, nitro, halogen, nitrile, sulfonic acid and carboxy; and Z is the residue of a compound represented by the formula



35

in which R5 is one of a group consisting of hydrogen, alkyl, alkoxy, phenyl-alkoxy, hydroxy, amino, alkylated amino, halogen, CN and sulfonic acid, and the R4 groups are like or different members of a group consisting of amino, alkylated amino and hydroxy.

3. A compound represented by the formula

50



55

in which R1 is from the group consisting of hydrogen, alkyl, alkoxy and halogen; n is an integer not greater than 2; Y is the residue of an amino naphthol sulfonic acid represented by the formula



60

in which amino is in one of the positions 1 and 2 and R3 is one of a group consisting of hydrogen, alkyl, alkoxy, aralkyl, nitro, halogen, nitrile, sulfonic acid and carboxy; and Z is the residue of a compound represented by the formula



65

in which R is one of a group consisting of hydro-

75

gen, alkyl, phenyl-alkyl, alkoxy, hydroxy, amino, alkylated amino, halogen, CN and sulfonic acid, and the  $R_4$  groups are like or different members of a group consisting of amino, alkylated amino and hydroxy.

4. A compound represented by the formula



in which **X** is the residue after tetrazotization of a diphenylene diamine in which the amino groups are in meta or para positions to the bridged carbons and are represented by the formula



20 in which B is one of a group consisting of  $-\text{O}-$ ,  
 $-\text{S}-$ ,  $-\text{NH}-$ ,  $-\text{NHCONH}-$ ,  $-\text{NHCSNH}-$ ,  
 $-\text{CONH}-$ ,  $-\text{CONH}(\text{CH}_2)_m\text{NHCO}-$ ,  $-\text{HC=}$   
 $\text{CH}-$



30 wherein the  $-\text{NHCO}-$  groups are meta or para to each other,  $-\text{O}(\text{CH}_2)_m\text{O}-$ ,  $-\text{S}(\text{CH}_2)_m\text{S}-$ ,  $-\text{N}=\text{N}-$ .



35 and  $-(\text{CH}_2)_m-$ ,  $n$  is an integer not greater than 2,  $m$  is 2 to 7,  $R_1$  is from the group consisting of hydrogen, alkyl, alkoxy and halogen and  $R_2$  is from the group consisting of hydrogen, alkyl, alkoxy and halogen;  $Y$  is the residue of an amino naphthol sulfonic acid represented by the formula



in which amino is in one of the positions 1 and 2 and R<sub>3</sub> is one of a group consisting of hydrogen, alkyl, alkoxy, aralkyl, nitro, halogen, nitrile, sulfonyl acid and carboxyl.

50 5. The compound represented by the formula:



6. The formaldehyde complexes of the compounds of claim 1.

7. The formaldehyde complexes of the compounds of claim 2.

70 8. The formaldehyde complexes of the compounds of claim 3.

9. The formaldehyde complexes of the compounds of claim 5.

10. The formaldehyde and metal complexes of  
75 the compounds of claim 1.

11. The formaldehyde and metal complexes of the compounds of claim 2.
  12. The formaldehyde and metal complexes of the compounds of claim 3.
  13. The formaldehyde and metal complexes of the compounds of claim 5.

14. The process which comprises diazotizing a compound Y which is represented by the formula



in which amino is in one of the positions 1 and 2 15  
 and  $R_3$  is one of a group consisting of hydrogen, alkyl, alkoxy, aralkyl, nitro, halogen, nitrile, sulfonic acid and carboxy; coupling with an equimolecular proportion of a compound Z which is represented by the formula. 20



in which R is one of a group consisting of hydrogen, alkyl, alkoxy, phenyl-alkyl, hydroxy, amino, alkylated amino, halogen, CN and sulfonic acid, and the R<sub>4</sub> groups are at least one of a group consisting of amino, alkylated amino and hydroxy; separating the product of coupling Y→Z from the coupling medium and making a dilute basic solution thereof; tetrazotizing about two mol equivalents of a compound X which is represented by the formula



in which B is one of a group consisting of  $-\text{O}-$ ,  $-\text{S}-$ ,  $-\text{NH}-$ ,  $-\text{NHCONH}-$ ,  $-\text{NHCSNH}-$ ,  $-\text{CONH}-$ ,  $-\text{CONH}(\text{CH}_2)_m\text{NHCO}-$ ,  $-\text{HC=CH}-$



wherein the  $-\text{NHCO}-$  groups are meta or para. 50

to each other,  $-\text{O}(\text{CH}_2)_m\text{O}-$ ,  $-\text{S}(\text{CH}_2)_m\text{S}-$ ,  $-\text{N}=\text{N}-$ .



and  $-(\text{CH}_2)_m-$ ,  $n$  is an integer not greater than 2,  $m$  is 2 to 7,  $R_1$  is from the group consisting of hydrogen, alkyl, alkoxy and halogen and  $R_2$  is from the group consisting of hydrogen, alkyl, alkoxy and halogen; coupling said tetrazo with

said compound Y→Z; tetrazotizing the resulting compound X→Y→Z→X and coupling with about two mol equivalents of a meta-dihydroxy benzene which is represented by the formula

5



10 in which R is one of a group consisting of hydrogen, alkyl, alkoxy, aralkyl, hydroxy, amino, halogen, nitrile, carboxy and sulfonic acid; and then separating the product of coupling from the coupling mixture.

15 15. The process which comprises dyeing a textile fabric with a compound represented by the formula



20 in which A is the residue after coupling of a meta-dihydroxy benzene represented by the formula

25



30 in which R is one of a group consisting of hydrogen, alkyl, alkoxy, aralkyl, hydroxy, amino, halogen, nitrile, carboxy and sulfonic acid; each X is the residue after tetrazotization of a diphenylene diamine compound in which the amino groups are in meta or para positions to the bridged carbons and are represented by the formula

35



40 40. in which B is one of a group consisting of —O—, —S—, —NH—, —NHCONH—, —NHCSNH—, —CONH—, —(CONH(CH<sub>2</sub>)<sub>m</sub>NHCO)—, —HC=CH—

45



50 50. wherein the —NHCO— groups are meta or para to each other, —O(CH<sub>2</sub>)<sub>m</sub>O—, —S(CH<sub>2</sub>)<sub>m</sub>S—, —N=N—,



55 55. and —(CH<sub>2</sub>)<sub>m</sub>—, n is an integer not greater than 2, m is 2 to 7, R<sub>1</sub> is from the group consisting of hydrogen, alkyl, alkoxy and halogen and R<sub>2</sub> is from the group consisting of hydrogen, alkyl, alkoxy and halogen; Y is the residue of an amino naphthol sulfonic acid represented by the formula

65



in which amino is in one of the positions 1 and 2 and R<sub>3</sub> is one of a group consisting of hydrogen,

alkyl, alkoxy, aralkyl, nitro, halogen, nitrile, sulfonic acid and carboxy; and Z is the residue of a compound represented by the formula

5



10 in which R<sub>5</sub> is one of a group consisting of hydrogen, alkyl, alkoxy, phenyl-alkyl, hydroxy, amino, alkylated amino, halogen, CN and sulfonic acid, and the R<sub>4</sub> is at least one of the group consisting of amino, alkylated amino and hydroxy; suspending the dyed fabric in a hydrous bath containing at least sufficient formaldehyde to form a formaldehyde complex with the compound on the fiber; and heating until said formaldehyde complex is formed.

15 16. The process in accordance with claim 15 in which the dyed fabric is treated consecutively with first one and then the other of the group of compounds consisting of formaldehyde and a soluble metal salt of a metal having an atomic weight between 50 and 65 until a metal and formaldehyde complex is formed.

20 17. The compound represented by the formula:



30

35

40

45

18. The compound represented by the formula:



50

55

60

SWANIE S. ROSSANDER,  
CHILES E. SPARKS.